

(No Model.)

H. A. ROWLAND.

CASTING BRASS AND OTHER METALS.

No. 272,088.

Patented Feb. 13, 1883.



WITNESSES:

D. Day Paul,  
D. Cowan.

*Henry A. Rowland*  
INVENTOR.

By *A. Stewart*  
Attorney.

# UNITED STATES PATENT OFFICE.

HENRY A. ROWLAND, OF BALTIMORE, MARYLAND.

## CASTING BRASS AND OTHER METALS.

SPECIFICATION forming part of Letters Patent No. 272,088, dated February 13, 1883.

Application filed December 16, 1882. (No model.)

*To all whom it may concern:*

Be it known that I, HENRY A. ROWLAND, of Baltimore city, State of Maryland, have invented certain new and useful Improvements 5 in Casting Brass and other Metals; and I do hereby declare that the following is a full, clear, and exact description thereof, reference being had to the accompanying drawings, and the letters of reference marked thereon, which 10 form a part of this specification.

In the drawings, Figure 1 is a sectional view 15 of a mold for casting plates of metal for any purpose. Fig. 2 is a perspective view of the same mold without the cover B. Fig. 3 is a section of the hinge C.

A is a box-mold, with a cover, B, hinged at C.

D is a pipe communicating with a gasometer 20 and passing through the cover B at F.

E is the mouth of the mold, provided with a funnel for the better pouring of the metal.

G is a neck or trough let into the side of the mold at H and rising to the level of the cover B at E.

25 Manufacturers have found by experience that in order to get a perfectly homogeneous casting with any of the metals that unite readily with oxygen when melted it is necessary to produce two conditions: first, an atmosphere into which the metal is poured that will be free from oxygen, and, secondly, a means by which any oxide of the metal which has formed upon it before it reaches the mold may be reduced. Various means have been devised for these purposes; but in all of them the 30 two conditions were the result of separate and distinct operations invented at different times and used independently of one another.

Now, the subject of my invention and the 40 thing of which I believe myself to be the first inventor is a method by which these two conditions are produced at the same time, by one operation and the use of one material, with great economy of both time and material, and 45 producing much more certain results than it

has been possible to attain by any of the methods heretofore in use.

My invention consists in forcing into a mold in which metal is to be cast a stream of ordinary illuminating-gas or any other inflammable deoxidizing-gas, as shown in the drawings at D, in such a manner that it will first fill it, thereby expelling the oxygen, and then flow out at the mouth. When the molten metal is poured it will ignite the gas at E, as it escapes 55 from the mold, as soon as it comes into contact with it, and thus produce the reducing-flame I, through which the metal must pass on its way into the mold. After passing the flame at E the molten metal flows down the 60 inclined gutter G before reaching the mold, and any oxide that may have failed to be reduced by the flame at E will either be driven back toward E by the force of the stream of gas that is flowing over its surface or be reduced by the waste heat of the molten metal, 65 the atmosphere being free from oxygen.

I do not claim to be the inventor of casting metal in an atmosphere of deoxidizing-gas, nor am I the inventor of the method of reducing 70 the oxide of metal by the use of a flame at the mouth of the mold; but I believe myself to be the first one who has ever used the ordinary illuminating-gas or any other inflammable deoxidizing-gas to accomplish both purposes by 75 one operation, and that this is the cheapest and best method devised for the purpose.

What I claim, therefore, as my invention is—

The above-described method of casting metal by first forcing illuminating-gas or any other 80 inflammable deoxidizing-gas into a mold, so as to expel the air therefrom and occupy its place, and then pouring the metal through the ignited gas as it escapes from the mouth of the mold, substantially as described, for the purpose set 85 forth.

HENRY A. ROWLAND.

Witnesses:

ARTHUR STEUART,  
JAMES L. STEUART.